



US006456812B1

(12) **United States Patent**  
Gervasi et al.

(10) **Patent No.:** US 6,456,812 B1  
(45) **Date of Patent:** Sep. 24, 2002

(54) **COATING COMPOSITIONS FOR  
DEVELOPMENT ELECTRODES**

(75) Inventors: **David J. Gervasi**, West Henrietta;  
**Yelena Shapiro**, Rochester; **Kip L. Jugle**, Bloomfield; **Santokh S. Badesha**, Pittsford; **George J. Bingham**, Webster; **William H. Wayman**, Ontario, all of NY (US)

(73) Assignee: **Xerox Corporation**, Stamford, CT (US)

(\*) Notice: Subject to any disclaimer, the term of this patent is extended or adjusted under 35 U.S.C. 154(b) by 79 days.

(21) Appl. No.: **09/654,778**

(22) Filed: **Sep. 5, 2000**

(51) Int. Cl.<sup>7</sup> ..... **G03G 15/08**

(52) U.S. Cl. ..... **399/266**

(58) Field of Search ..... 399/266; 428/36.91,  
428/36.9

(56) **References Cited**

U.S. PATENT DOCUMENTS

|             |           |                     |          |
|-------------|-----------|---------------------|----------|
| 4,868,600 A | 9/1989    | Hays et al. ....    | 355/259  |
| 4,984,019 A | 1/1991    | Folkins ....        | 355/215  |
| 5,124,749 A | 6/1992    | Bares ....          | 355/202  |
| 5,172,170 A | 12/1992   | Hays et al. ....    | 355/259  |
| 5,300,339 A | 4/1994    | Hays et al. ....    | 428/36.9 |
| 5,448,342 A | 9/1995    | Hays et al. ....    | 355/259  |
| 5,848,327 A | * 12/1998 | Badesha et al. .... | 399/266  |
| 5,999,781 A | * 12/1999 | Gervasi et al. .... | 399/266  |

\* cited by examiner

Primary Examiner—Alexander S. Thomas

(74) Attorney, Agent, or Firm—Anette L. Bade

(57) **ABSTRACT**

An improved apparatus and process for reducing accumulation of toner from the surface of an electrode member in a development unit of an electrostatographic printing apparatus by providing a composition coating comprising a water-emulsified polymer, lubricant and inorganic material on at least a portion of the electrode member.

**21 Claims, 3 Drawing Sheets**





**FIG. 1**



FIG. 2



FIG. 3

**FIG.4****FIG.5**

## COATING COMPOSITIONS FOR DEVELOPMENT ELECTRODES

### BACKGROUND OF THE INVENTION

The present invention relates to methods, processes and apparatus for development of images, and more specifically, to electrode members for use in a developer unit in electrostatographic printing or copying machines, or in digital imaging systems such as the Xerox Corporation 220 and 230 machines. Specifically, the present invention relates to apparatus in which at least a portion of a development unit electrode member is coated with a coating composition, and in embodiments, a low surface energy coating. In embodiments, electrode member history, damping and/or toner accumulation is controlled or reduced.

Generally, the process of electrostatographic printing or copying includes charging a photoconductive member to a substantially uniform potential so as to sensitize the photoconductive member thereof. The charged portion of the photoconductive member is exposed to a light image of an original document being reproduced. This records an electrostatic latent image on the photoconductive member. After the electrostatic latent image is recorded on the photoconductive member, the latent image is developed by bringing a developer into contact therewith. Two component and single component developers are commonly used. A typical two component developer comprises magnetic carrier granules having toner particles adhering triboelectrically thereto. A single component developer typically comprises toner particles. Toner particles are attracted to the latent image forming a toner powder image on the photoconductive member. The toner powder image is subsequently transferred to a copy sheet. Finally, the toner powder image is heated to permanently fuse it to the copy sheet in image configuration.

One type of single component development system is a scavengerless development system that uses a donor roll for transporting charged toner to the development zone. At least one, and preferably a plurality of electrode members are closely spaced to the donor roll in the development zone. An AC voltage is applied to the electrode members forming a toner cloud in the development zone. The electrostatic fields generated by the latent image attract toner from the toner cloud to develop the latent image.

Another type of a two component development system is a hybrid scavengerless development system, which employs a magnetic brush developer roller for transporting carrier having toner adhering triboelectrically thereto. A donor roll is used in this configuration also to transport charged toner to the development zone. The donor roll and magnetic roller are electrically biased relative to one another. Toner is attracted to the donor roll from the magnetic roll. The electrically biased electrode members detach the toner from the donor roll forming a toner powder cloud in the development zone, and the latent image attracts the toner particles thereto. In this way, the latent image recorded on the photoconductive member is developed with toner particles.

Various types of development systems have hereinbefore been used as illustrated by the following:

U.S. Pat. No. 4,868,600 to Hays et al., the subject matter of which is hereby incorporated by reference in its entirety, describes an apparatus wherein a donor roll transports toner to a region opposed from a surface on which a latent image is recorded. A pair of electrode members are positioned in the space between the latent image surface and the donor roll and are electrically biased to detach toner from the donor roll

to form a toner cloud. Detached toner from the cloud develops the latent image.

U.S. Pat. No. 4,984,019, to Folkins, the subject matter of which is hereby incorporated by reference in its entirety, discloses a developer unit having a donor roll with electrode members disposed adjacent thereto in a development zone. A magnetic roller transports developer material to the donor roll. Toner particles are attracted from the magnetic roller to the donor roller. When the developer unit is inactivated, the electrode members are vibrated to remove contaminants therefrom.

U.S. Pat. No. 5,124,749 to Bares, the subject matter of which is hereby incorporated by reference in its entirety, discloses an apparatus in which a donor roll advances toner to an electrostatic latent image recorded on a photoconductive member wherein a plurality of electrode wires are positioned in the space between the donor roll and the photoconductive member. The wires are electrically biased to detach the toner from the donor roll so as to form a toner cloud in the space between the electrode wires and the photoconductive member. The powder cloud develops the latent image. A damping material is coated on a portion of the electrode wires at the position of attachment to the electrode supporting members for the purpose of damping vibration of the electrode wires.

U.S. Pat. Nos. 5,300,339 and 5,448,342 both to Hays et al., the subject matter each of which is hereby incorporated by reference in their entirety, disclose a coated toner transport roll containing a core with a coating thereover.

U.S. Pat. No. 5,172,170 to Hays et al., the subject matter of which is hereby incorporated by reference in its entirety, discloses an apparatus in which a donor roll advances toner to an electrostatic latent image recorded on a photoconductive member. The donor roll includes a dielectric layer disposed about the circumferential surface of the roll between adjacent grooves.

Primarily because the adhesion force of the toner particles is greater than the stripping force generated by the electric field of the electrode members in the development zone, a toner tends to build up on the electrode members. Accumulation of toner particles on the wire member causes non-uniform development of the latent image, resulting in print defects. This problem is aggravated by toner fines and any toner components, such as high molecular weight, crosslinked and/or branched components, and the voltage breakdown between the wire member and the donor roll.

One specific example of toner contamination results upon development of a document having solid areas that require a large concentration of toner to be deposited at a particular position on the latent image. The areas of the electrode member corresponding to the high throughput or high toner concentration areas tend to include higher or lower accumulation of toner because of this differing exposure to toner throughput. When subsequently attempting to develop another, different image, the toner accumulation on the electrode member can lead to differential development of the newly developed image corresponding to the areas of greater or lesser toner accumulation on the electrode members. The result is a darkened or lightened band in the position corresponding to the solid area of the previous image. This is particularly evident in areas of intermediate density, since these are the areas most sensitive to differences in development. These particular image defects caused by toner accumulation on the electrode wires at the development zone are referred to as wire history. FIG. 5 contains an illustration of wire contamination and wire history. Wire contamination

results when fused toner forms between the electrode member and donor member due to toner fines and any toner components, such as high molecular weight, cross-linked and/or branched components, and the voltage breakdown between the wire member and the donor roll. Wire history is a change in develop-ability due to toner or toner components sticking to the top of the electrode member.

Accordingly, there is a specific need for electrode members in the development zone of a development unit of an electrophotographic printing or copying machine which provide for a decreased tendency for toner accumulation to thereby primarily decrease wire history and wire contamination, especially at high throughput areas, and decreasing the production of unwanted surface static charges from which contaminants may not release. One possible solution is to change the electrical properties of the wire. However, attempts at decreasing toner build-up on the development wire by changing the electrical properties thereof, may result in an interference with the function of the wire and its ability to produce the formation of the toner powder cloud. Therefore, there is a specific need for electrode members which have a decreased tendency to accumulate toner and which also retain their electrical properties in order to prevent interference with the functioning thereof. There is an additional need for electrode members which have superior mechanical properties including durability against severe wear the electrode member receives when it is repeatedly brought into contact with tough rotating donor roll surfaces.

U.S. Pat. No. 5,761,587 discloses an electrode member having a coating on at least a portion of nonattached regions of the electrode member.

U.S. Pat. No. 5,787,329 discloses an electrode member having a low surface energy organic coating on at least a portion of nonattached regions of the electrode member.

U.S. Pat. No. 5,805,964 discloses an electrode member having an inorganic coating on at least a portion of nonattached regions of the electrode member.

U.S. Pat. No. 5,778,290 discloses an electrode member having a composite coating on at least a portion of nonattached regions of the electrode member

U.S. Pat. No. 5,848,327 discloses an electrode member having a composition coating on at least a portion of nonattached regions of the electrode member.

U.S. Pat. No. 5,999,781 discloses an electrode member having a composition coating on at least a portion of nonattached regions of the electrode member, wherein the composition comprises a polymer, lubricant and inorganic material.

Wire history and wire contamination were reduced by use of the above coating formulations to some extent. However, the above formulations were found to have several limitations. First, the liquid coating dispersions contained volatile organic solvents, which were shown to be disagreeable to several coating applicators under increasing environmental restrictions. Second, while the coatings reduced wire history defects significantly as compared to uncoated stainless steel wires, the coatings were not shown to reduce the defect to below visible levels.

Therefore, there still exists a need for a wire coating that reduces wire defect and wire contamination to below visible levels. In addition, there is a need for a wire coating which is environmentally friendly. A need further remains for electrode members which have superior mechanical properties including durability against severe wear the electrode member receives when it is repeatedly brought into contact with tough rotating donor roll surfaces.

## SUMMARY OF THE INVENTION

The present invention includes, in embodiments, an improved apparatus for developing a latent image recorded on a surface, of the type comprising: wire supports; a donor member spaced from the surface and being adapted to transport toner to a region opposed from the surface; and an electrode member positioned in the space between the surface and the donor member, the electrode member being closely spaced from the donor member and being electrically biased to detach toner from the donor member thereby enabling the formation of a toner cloud in the space between the electrode member and the surface with detached toner from the toner cloud developing the latent image, wherein opposed end regions of the electrode member are attached to said wire supports adapted to support the opposed end regions of said electrode member; wherein the improvement comprises a coating composition comprising a water-emulsified polymer, a lubricant and an inorganic material on at least a portion of nonattached regions of said electrode member.

Embodiments further include: an improved apparatus for developing a latent image recorded on a surface, of the type comprising: wire supports; a donor member spaced from the surface and being adapted to transport toner to a region opposed from the surface; and an electrode member positioned in the space between the surface and the donor member, the electrode member being closely spaced from the donor member and being electrically biased to detach toner from the donor member thereby enabling the formation of a toner cloud in the space between the electrode member and the surface with detached toner from the toner cloud developing the latent image, wherein opposed end regions of the electrode member are attached to said wire supports adapted to support the opposed end regions of said electrode member; the improvement comprising a coating composition comprising a water-emulsified poly (amide-imide) polymer, a fluorinated ethylene propylene lubricant and carbon black on at least a portion of nonattached regions of said electrode member.

In addition, embodiments of the present invention include: an improved electrostatographic process of the type comprising: a) forming an electrostatic latent image on a charge-retentive surface; b) applying toner in the form of a toner cloud to said latent image to form a developed image on said charge retentive surface, wherein said toner is applied using a development apparatus comprising wire supports; a donor member spaced from the surface and being adapted to transport toner to a region opposed from the surface; an electrode member positioned in the space between the surface and said donor member, said electrode member being closely spaced from said donor member and being electrically biased to detach toner from said donor member thereby enabling the formation of a toner cloud in the space between said electrode member and the surface with detached toner from the toner cloud developing the latent image, wherein opposed end regions of said electrode member are attached to said wire supports adapted to support the opposed end regions of said electrode member; wherein the improvement comprises a water-emulsified polymer, a lubricant, and an inorganic material on at least a portion of nonattached regions of said electrode member; c) transferring the toner image from said charge-retentive surface to a substrate; and d) fixing said toner image to said substrate.

The present invention provides electrode members which, in embodiments, have a decreased tendency to accumulate

toner and which also, in embodiments, retain their electrical properties in order to prevent interference with the functioning thereof. The present invention further provides electrode members which, in embodiments, have superior mechanical properties including durability against severe wear the electrode member receives when it is repeatedly brought into contact with tough rotating donor roll surfaces. The present invention also provides electrode members having an outer coating which is environmentally friendly.

#### BRIEF DESCRIPTION OF THE DRAWINGS

The above aspects of the present invention will become apparent as the following description proceeds upon reference to the drawings in which:

FIG. 1 is a schematic illustration of an embodiment of a development apparatus useful in an electrophotographic printing machine.

FIG. 2 is an enlarged, schematic illustration of a donor roll and electrode member representing an embodiment of the present invention.

FIG. 3 is a fragmentary schematic illustration of a development housing comprising a donor roll and an electrode member from a different angle than as shown in FIG. 2.

FIG. 4 is an enlarged, schematic illustration of an electrode member supported by mounting means in an embodiment of the present invention.

FIG. 5 is an illustration of wire contamination and wire history.

#### DETAILED DESCRIPTION

For a general understanding of the features of the present invention, a description thereof will be made with reference to the drawings.

FIG. 1 shows a development apparatus used in an electrostatographic printing machine such as that illustrated and described in U.S. Pat. No. 5,124,749, the disclosure of which is hereby incorporated by reference in its entirety. This patent describes the details of the main components of an embodiment of an electrostatographic printing machine and how these components interact. The present application will concentrate on the development unit of the electrophotographic printing machine. Specifically, after an electrostatic latent image has been recorded on a photoconductive surface, a photoreceptor belt advances the latent image to the development station. At the development station, a developer unit develops the latent image recorded on the photoconductive surface.

Referring now to FIG. 1, in a preferred embodiment of the invention, developer unit 38 develops the latent image recorded on the photoconductive surface 10. Preferably, developer unit 38 includes donor roller 40 and electrode member or members 42. Electrode members 42 are electrically biased relative to donor roll 40 to detach toner therefrom so as to form a toner powder cloud in the gap between the donor roll 40 and photoconductive surface 10. The latent image attracts toner particles from the toner powder cloud forming a toner powder image thereon. Donor roller 40 is mounted, at least partially, in the chamber of developer housing 44. The chamber in developer housing 44 stores a supply of developer material. The developer material is a two component developer material of at least carrier granules having toner particles adhering triboelectrically thereto. A magnetic roller 46 disposed interior of the chamber of housing 44 conveys the developer material to the donor roller 40. The magnetic roller 46 is electrically biased

relative to the donor roller so that the toner particles are attracted from the magnetic roller to the donor roller.

More specifically, developer unit 38 includes a housing 44 defining a chamber 76 for storing a supply of two component (toner and carrier) developer material therein. Donor roller 40, electrode members 42 and magnetic roller 46 are mounted in chamber 76 of housing 44. The donor roller can be rotated in either the 'with' or 'against' direction relative to the direction of motion of belt 10. In FIG. 1, donor roller 40 is shown rotating in the direction of arrow 68. Similarly, the magnetic roller can be rotated in either the 'with' or 'against' direction relative to the direction of motion of belt 10. In FIG. 1, magnetic roller 46 is shown rotating in the direction of arrow 92. Donor roller 40 is preferably made from anodized aluminum or ceramic.

Developer unit 38 also has electrode members 42 which are disposed in the space between the belt 10 and donor roller 40. A pair of electrode members are shown extending in a direction substantially parallel to the longitudinal axis of the donor roller. The electrode members are made from of one or more thin (i.e., 50 to 100  $\mu\text{m}$  in diameter) stainless steel or tungsten electrode members which are closely spaced from donor roller 40. The distance between the electrode members and the donor roller is from about 0.001 to about 45  $\mu\text{m}$ , preferably about 10 to about 25  $\mu\text{m}$  or the thickness of the toner layer on the donor roll. The electrode members are self-spaced from the donor roller by the thickness of the toner on the donor roller. To this end, the extremities of the electrode members supported by the tops of end bearing blocks also support the donor roller for rotation. The electrode member extremities are attached so that they are slightly above a tangent to the surface, including toner layer, of the donor structure. Mounting the electrode members in such a manner makes them insensitive to roll run-out due to their self-spacing.

As illustrated in FIG. 1, an alternating electrical bias is applied to the electrode members by an AC voltage source 78. The applied AC establishes an alternating electrostatic field between the electrode members and the donor roller is effective in detaching toner from the photoconductive member of the donor roller and forming a toner cloud about the electrode members, the height of the cloud being such as not to be substantially in contact with the belt 10. The magnitude of the AC voltage is relatively low and is in the order of about 200 to about 500 volts peak at a frequency ranging from about 9 kHz to about 15 kHz. A DC bias supply 80 which applies approximately 300 volts to donor roller 40 establishes an electrostatic field between photoconductive member of belt 10 and donor roller 40 for attracting the detached toner particles from the cloud surrounding the electrode members to the latent image recorded on the photoconductive member. At a spacing ranging from about 0.001  $\mu\text{m}$  to about 45  $\mu\text{m}$  between the electrode members and donor roller, an applied voltage of about 200 to about 500 volts produces a relatively large electrostatic field without risk of air breakdown. A cleaning blade 82 strips all of the toner from donor roller 40 after development so that magnetic roller 46 meters fresh toner to a clean donor roller. Magnetic roller 46 meters a constant quantity of toner having a substantially constant charge onto donor roller 40. This insures that the donor roller provides a constant amount of toner having a substantially constant charge in the development gap. In lieu of using a cleaning blade, the combination of donor roller spacing, i.e., spacing between the donor roller and the magnetic roller, the compressed pile height of the developer material on the magnetic roller, and the magnetic properties of the magnetic roller in conjunction

with the use of a conductive, magnetic developer material achieves the deposition of a constant quantity of toner having a substantially charge on the donor roller. A DC bias supply 84 which applies approximately 100 volts to magnetic roller 46 establishes an electrostatic field between magnetic roller 46 and donor roller 40 so that an electrostatic field is established between the donor roller and the magnetic roller which causes toner particles to be attracted from the magnetic roller to the donor roller. Metering blade 86 is positioned closely adjacent to magnetic roller 46 to maintain the compressed pile height of the developer material on magnetic roller 46 at the desired level. Magnetic roller 46 includes a non-magnetic tubular member 88 made preferably from aluminum and having the exterior circumferential surface thereof roughened. An elongated magnet 90 is positioned interiorly of and spaced from the tubular member. The magnet is mounted stationarily. The tubular member rotates in the direction of arrow 92 to advance the developer material adhering thereto into the nip defined by donor roller 40 and magnetic roller 46. Toner particles are attracted from the carrier granules on the magnetic roller to the donor roller.

With continued reference to FIG. 1, an auger, indicated generally by the reference numeral 94, is located in chamber 76 of housing 44. Auger 94 is mounted rotatably in chamber 76 to mix and transport developer material. The auger has blades extending spirally outwardly from a shaft. The blades are designed to advance the developer material in the axial direction substantially parallel to the longitudinal axis of the shaft.

As successive electrostatic latent images are developed, the toner particles within the developer are depleted. A toner dispenser (not shown) stores a supply of toner particles which may include toner and carrier particles. The toner dispenser is in communication with chamber 76 of housing 44. As the concentration of toner particles in the developer is decreased, fresh toner particles are furnished to the developer in the chamber from the toner dispenser. In an embodiment of the invention, the auger in the chamber of the housing mix the fresh toner particles with the remaining developer so that the resultant developer therein is substantially uniform with the concentration of toner particles being optimized. In this way, a substantially constant amount of toner particles are present in the chamber of the developer housing with the toner particles having a constant charge. The developer in the chamber of the developer housing is magnetic and may be electrically conductive. By way of example, in an embodiment of the invention wherein the toner includes carrier particles, the carrier granules include a ferromagnetic core having a thin layer of magnetite overcoated with a non-continuous layer of resinous material. The toner particles may be generated from a resinous material, such as a vinyl polymer, mixed with a coloring material, such as chromogen black. The developer may comprise from about 90% to about 99% by weight of carrier and from 10% to about 1% by weight of toner. However, one skilled in the art will recognize that any other suitable developers may be used.

In an alternative embodiment of the present invention, one component developer comprised of toner without carrier may be used. In this configuration, the magnetic roller 46 is not present in the developer housing. This embodiment is described in more detail in U.S. Pat. No. 4,868,600, the disclosure of which is hereby incorporated by reference in its entirety.

An embodiment of the developer unit is further depicted in FIG. 2. The developer apparatus 34 comprises an electrode member 42 which is disposed in the space between the

photoreceptor (not shown in FIG. 2) and the donor roll 40. The electrode 42 can be comprised of one or more thin (i.e., about 50 to about 100  $\mu\text{m}$  in diameter) tungsten or stainless steel electrode members, which are lightly positioned at or near the donor structure 40. The electrode member is closely spaced from the donor member. The distance between the wire(s) and the donor is approximately 0.001 to about 45  $\mu\text{m}$ , and preferably from about 10 to about 25  $\mu\text{m}$  or the thickness of the toner layer 43 on the donor roll. The wires as shown in FIG. 2 are self spaced from the donor structure by the thickness of the toner on the donor structure. The extremities or opposed end regions of the electrode member are supported by support members 54 that may also support the donor structure for rotation. In a preferred embodiment, the electrode member extremities or opposed end regions are attached so that they are slightly below a tangent to the surface, including toner layer, of the donor structure. Mounting the electrode members in such a manner makes them insensitive to roll run-out due to the self-spacing.

In an alternative embodiment to that depicted in FIG. 1, the metering blade 86 is replaced by a combined metering and charging blade 86 as shown in FIG. 3. The combination metering and charging device may comprise any suitable device for depositing a mono-layer of well-charged toner onto the donor structure 40. For example, it may comprise an apparatus such as that described in U.S. Pat. No. 4,459,009, wherein the contact between weakly charged toner particles and a triboelectrically active coating contained on a charging roller results in well charged toner. Other combination metering and charging devices may be employed, for example, a conventional magnetic brush used with two component developer could also be used for depositing the toner layer onto the donor structure, or a donor roller alone used with one component developer.

FIG. 4 depicts an enlarged view of a preferred embodiment of the electrode member of the present invention. Electrode wires 45 are positioned inside electrode member 42. The anchoring portions 55 of the electrode members are the portions of the electrode member, which anchor the electrode member to the support member. The mounting sections 56 of the electrode member are the sections of the electrode members between the electrode member and the mounting means 54.

Toner particles are attracted to the electrode members primarily through electrostatic attraction. Toner particles adhere to the electrode members because the adhesion force of the toner is larger than the stripping force generated by the electric field of the electrode member. Generally, the adhesion force between a toner particle and an electrode member is represented by the general expression  $F_{ad}=q^2/kr_2+W$ , wherein  $F_{ad}$  is the force of adhesion,  $q$  is the charge on the toner particle,  $k$  is the effective dielectric constant of the toner and any dielectric coating, and  $r$  is the separation of the particle from its image charge within the wire which depends on the thickness, dielectric constant, and conductivity of the coating. Element  $W$  is the force of adhesion due to short range adhesion forces such as van der Waals and capillary forces. The force necessary to strip or remove particles from the electrode member is supplied by the electric field of the wire during half of its AC period,  $qE$ , plus effective forces resulting from mechanical motion of the electrode member and from bombardment of the wire by toner in the cloud. Since the adhesion force is quadratic in  $q$ , adhesion forces will be larger than stripping forces.

FIG. 5 contains an illustration of wire contamination and wire history. A photoreceptor 1 is positioned near wire 4 and contains an undeveloped image 6 which is subsequently

developed by toner originating from donor member 3. Wire contamination occurs when fused toner 5 forms between the wire 4 and donor member 3. The problem is aggravated by toner fines and any toner components, such as high molecular weight, cross-linked and/or branched components, and the voltage breakdown between the wire member and the donor roll. Wire history is a change in develop-ability due to toner 2 or toner components sticking to the top of the wire 4, the top of the wire being the part of the wire facing the photoreceptor.

In order to prevent the toner defects associated with wire contamination and wire history, the electrical properties of the electrode member can be changed, thereby changing the adhesion forces in relation to the stripping forces. However, such changes in the electrical properties of the electrode member may adversely affect the ability of the electrode member to adequately provide a toner cloud, which is essential for developing a latent image. The present invention is directed to an apparatus for reducing the unacceptable accumulation of toner on the electrode member while maintaining the desired electrical and mechanical properties of the electrode member. The electrode member of the present invention is coated with a material coating that reduces the significant attraction of toner particles to the electrode member, which may result in toner accumulation. However, the material coating does not adversely interfere with the mechanical or electrical properties of the electrode member.

The present materials decrease or eliminate wire history defects to where the defect is below visible levels. The present materials have the added benefit of being environmentally friendly as they do not contain volatile organic solvents.

The improved composition decreases the accumulation of toner by assuring electrical continuity for charging the wires and eliminates the possibility of charge build-up. In addition, such improved materials as described herein do not interfere with the electrical properties of the electrode member and do not adversely affect the electrode's ability to produce a toner powder cloud. Moreover, the electrode member maintains its tough mechanical properties, allowing the electrode member to remain durable against the severe wear the electrode member receives when it is repeatedly brought into contact with tough, rotating donor roll surfaces. Also, the electrode member maintains a "smooth" surface after the coating is applied. A smooth surface includes surfaces having a surface roughness of less than about 5 microns, preferably from about 0.01 to about 1 micron.

In a preferred embodiment, the improved coating composition comprises a water-emulsified polymer, a lubricant and an inorganic material.

Water-emulsified, as used herein, refers to a polymeric dispersion that is incorporated into a liquid matrix comprised predominately of water, for example, from about 55 to about 95 and preferably from about 60 to about 90 percent water. While the polymer is not dissolved or solvated by water, it is a stable suspension of a polymer in water.

Preferred examples of water-emulsified polymers include water-emulsified resins such as water-emulsified poly (amide-imide), acrylic, epoxy-phenolic. The water-emulsified polymer contains reduced amounts of volatile organic solvents, and is therefore, environmentally friendly.

The water-emulsified polymer or polymers is present in the composition coating in a total amount of from about 25 to about 95 percent by weight, preferably from about 50 to about 90 percent by weight, and particularly preferred about 75 percent by weight of the total composition. Total

composition, as used herein, refers to the total amount by weight of water-emulsified polymer, lubricant and inorganic material, wherein the inorganic material may comprises in some embodiments, for example, reinforcer(s) and/or electrically conductive filler(s).

In a preferred embodiment, a lubricant is present in the coating composition. The primary purpose of the lubricant is to provide a non-sticky nature to the top surface of the coating so that the toner does not adhere to the electrode member. The lubricant preferably has the characteristics of relatively low porosity, relatively low coefficient of friction, thermal stability, relatively low surface energy, and possesses the ability to be relatively inert to chemical attack. Preferred examples of suitable lubricants include organic material such as, for example, fluoroplastic materials including TEFLON®-like materials such as polymers of tetrafluoroethylene (TFE) and polymers of fluorinated ethylene-propylene (FEP), such as, for example, polytetrafluoroethylene (PTFE), fluorinated ethylene-propylene copolymer (FEP), perfluorovinylalkylether tetrafluoroethylene copolymer (PFA TEFLON®), polyethersulfone, and copolymers thereof; and inorganic materials such as molybdenum disulfide, boron nitride, titanium diboride, graphite, and the like. In embodiments, a lubricant or mixture of lubricants, is present in a total amount of from about 3 to about 50 percent by weight, preferably from about 5 to about 25 percent by weight, and particularly preferred about 10 percent by weight of total coating composition.

In embodiments, the coating composition comprises an inorganic material. An inorganic filler can improve the composition toughness as well as tailor other properties such as color, and electrical and thermal conductivity of the polymer matrix. The added filler can also help to form a smooth surface for the coating composition. Examples of electrically conductive fillers include metal oxides such as tin oxide, titanium oxide, zirconium oxide, magnesium oxide and the like, and doped metal oxides such as antimony doped tin oxide, indium doped tin oxide, vanadium oxide and vanadium doped metal oxides, and the like. Another preferred filler is carbon black, graphite or the like, with surface treatment of compounds such as for example, siloxane, silane, fluorine or the like. Carbon Black is desired for its electrical conductivity and treating with surface fluorination can electrically insulate the carbon. Examples of suitable fillers include treated carbon blacks include fluorinated carbons such as those described in co-pending U.S. Pat. No. 6,130,061 the disclosure of which is hereby incorporated by reference in its entirety. More than one electrically conductive filler may be present in the coating composition. In preferred embodiments, an electrically conductive filler is present in a total amount of from about 5 to about 50 percent by weight, preferably from about 10 to about 25 percent by weight, and particularly preferred about 15 percent by weight of total composition.

In preferred embodiments, the polymer is a water-emulsified poly (amide-imide); the lubricant is fluorinated ethylene propylene; and the electrically conductive filler is carbon black. The resulting matrix includes the properties of all elements of the composition, including having high lubricity and low surface energy from the lubricant, having an overall high wear resistance due to the polymer component and reinforcers, and having a smooth surface and superior electrical properties due to the inorganic component including the reinforcer(s) and/or inorganic filler(s). The composition further decreases wire defect to below visible levels and is environmentally friendly.

The coating composition material including the water-emulsified polymer, lubricant and inorganic material, is

preferably present in an amount of from about 5 to about 95 percent by weight of total solids, and preferably from about 10 to about 40 percent by weight of total solids. Total solids refers to the total amount by weight of coating composition, solvent, optional fillers, and optional additives contained in the coating solution.

The volume resistivity of the coated electrode is, for example, from about  $10^{-10}$  to about  $1^{-1}$  ohm-cm, and preferably from  $10^{-5}$  to  $10^{-1}$  ohm-cm. The surface roughness is less than about 5 microns and preferably from about 0.01 to about 1 micron. The coating has a relatively low surface energy of from about 5 to about 35 dynes/cm, preferably from about 10 to about 25 dynes/cm.

In a preferred embodiment of the invention, the coating composition is coated over at least a portion of the nonattached regions of the electrode member. The nonattached region of the electrode member is the entire outer surface region of the electrode minus the region where the electrode is attached to the mounting means 54 and minus the anchoring area (55 in FIG. 4). It is preferred that the coating cover the portion of the electrode member which is adjacent to the donor roll. In another preferred embodiment of the invention, the coating composition is coated in an entire area of the electrode member located in a central portion of the electrode member and extending to an area adjacent to the nonattached portion of the electrode member. This area includes the entire surface of the electrode member minus the anchoring area (55 in FIG. 4). In an alternative embodiment, the entire length of the electrode member is coated with the material coating, including the anchoring area 55 and mounting area 56. In embodiments, at least a portion refers to the non-attached region being coated, or from about 10 to about 90 percent of the electrode member.

Toner can accumulate anywhere along the electrode member, but it will not affect development unless it accumulates in the length of the electrode member near to the donor roll or on the length closest to the photoreceptor. Therefore, it is preferred that the material coating cover the electrode member along the entire length corresponding to the donor roll, and on the entire length corresponding to the photoreceptor.

The coating composition may be deposited on at least a portion of the electrode member by any suitable, known method. These deposition methods include liquid and powder coating, dip and spray coating, and ion beam assisted and RF plasma deposition. In a preferred deposition method, the composition coating is coated on the electrode member by dip coating. After coating, the coating composition is preferably air dried and cured at a temperature suitable for curing the specific composition material. Curing temperatures range from about 100° F. to about 1400° F., and preferably from about 120° F. to about 1200° F.

The average thickness of the coating is from about 1 to about 30  $\mu\text{m}$  thick, and preferably from about 2 to about 10  $\mu\text{m}$  thick. If the coating is applied to only a portion of the electrode member, the thickness of the coating may or may not taper off at points farthest from the midpoint of the electrode member. Therefore, the thickness of the coating may decrease at points farther away from the midpoint of the electrode.

All the patents and applications referred to herein are hereby specifically, and totally incorporated herein by reference in their entirety in the instant specification.

The following Examples further define and describe embodiments of the present invention. Unless otherwise indicated, all parts and percentages are by weight.

## EXAMPLES

## Example 1

## Preparation of Wire to be Coated

5 A stainless steel wire of about 3 mil thickness was cleaned to remove obvious contaminants.

A dip coating apparatus consisting of a 1 inch (diameter) by 15 inches (length) glass cylinder sealed at one end to hold the liquid coating material was used for dip coating the wire. A cable attached to a Bodine Electric Company type NSH-10 12R motor was used to raise and lower a wire support holder that keeps the wire taut during the coating process. The dip and withdraw rate of the wire holder into and out of the coating solution was regulated by a motor control device from B&B Motors & Control Corporation, (NOVA PD DC motor speed control). After coating, a motor driven device was used to twirl the wire around its axis while it received external heating to allow for controlled solvent evaporation. When the coating was dry and/or non-flowable, the coated wire was heated in a flow through oven using a time and temperature schedule to complete either drying or cure/ post cure of the coating.

The general procedure may include: (A) cleaning and degreasing the wire with an appropriate solvent, for example, acetone, alcohol or water, and roughened if necessary by, for example, sand paper; (B) the coating material may be adjusted to the proper viscosity and solids content by adding solids or solvent to the solution; and (C) the wire is dipped into and withdrawn from the coating solution, dried and cured/post cured, if necessary, and dipped again, if required. The coating thickness and uniformity are a function of withdrawal rate and solution viscosity, (solids content in most solvent based systems) and a drying schedule consistent with the uniform solidification of the coating.

## Example 2

## Preparation of Composition Coating Solutions

A 2.5 mil stainless steel wire was prepared by lightly grit blasting, sanding or rubbing the wire surface with steel wool, degreasing with acetone and then rinsing with an isopropyl alcohol, and drying. The clean wire was primed with Whitford P-51 or Dow Coming 1200 primer using any convenient technique such as the conventional spray or dip/spin methods. The coating material was then applied. The coating material was D2340 (Xylan 1220/2810 Black) 45 supplied by Whitford Corporation, West Chester, Pa., which comprises a water-reducible poly (amide-imide) polymer resin that serves as a binder, about 15% by weight of carbon black which provides conductivity to the coating material, and an approximate 15% by weight loading of fluorinated ethylene propylene that lowers the surface energy of the coating material. The viscosity can be adjusted with deionized water to a 30 to 45 Zahn cup No. 2 immediately (a few seconds) before application. This dispersion was then dip coated onto an electrode as described in Example 1. A coating flash or air dry is optional; however to achieve optimum release, the cure time is preferably about 10 minutes at approximately 650° F. The coating can be polished to obtain a smooth and dry thickness of 2-3 microns thick.

60 Optionally, this coating composition can be coated on the electrode wire as in accordance with the procedures outlined in Example 1. The recommended dip application temperature is preferably between 70 and 80° F., and the desired application solution viscosity is between about 20 and 30 seconds using a Zahn No. 2. If a thinner coating is desired, water can be used as the diluent. The coated wire can be flashed for about 10 minutes at 400° F., and then baked for

## 13

about 20 minutes at approximately 750° F. This coating is expected to possess excellent adhesion and have a high wearability.

## Example 3

## Fixture Test of the Coated Electrode Wire

The wire coated with the coating composition of Example 2 was tested using various xerographic fixtures, which contained hybrid scavengeless development system described in detail above. Testing fixtures were comprised of entire electrostatographic printing machines, which included development, transfer, fuser and the like necessary components. Defects were generated by using approximately 1,000 pages of a "stress" document, followed by a different type of document referred to as "evaluation prints" for about 20 prints.

Most of the testing was preferred in monochrome mode, where wire history defect (mentioned above) or differential development was monitored on the evaluation prints. All testing was executed with consistent process parameters and materials packages. The only variable was the wire coating formulation. The results shown in Table 1 below demonstrate that by use of the coating composition herein performs unexpectedly superior as compared to previous coatings such as uncoated stainless steel, composition formulations using green pigmented polytetrafluoroethylene, and compositions using non water-reducible polymers.

Delta E was measured as a primary indicator of the level of defect between nominal and underdeveloped areas. Delta E is a difference between two points in the three-dimensional color space. Delta E was measured using an Xrite 964 spectrophotometer. Each reported delta E value is an average of several reads and several pages. Performance of over-coated and uncoated wires was judged based on delta E numbers. Lower values refer to less severe defect, and anything below dE=1 can be considered non-visible. Table 1 below shows the results of the testing. The results demonstrate that formulations comprising a water-emulsified polymer [solvent-borne poly(amide-imide)], lubricant [polytetrafluoroethylene (PTFE) or fluorinated ethylene propylene (FEP)] and inorganic material (carbon black) show dE values of less than 1, meaning that non-visible defects resulted.

TABLE 1

| Wire Coating ID             | Description                                              | dE   |
|-----------------------------|----------------------------------------------------------|------|
| Al#4                        | Solvent Borne Poly(amide-Imide) W/ Carbon Black and PTFE | 0.45 |
| Original Green D2342        | PTFE w/ Green Pigment                                    | 2.10 |
|                             | Water-borne Poly(amide-imide) w/ Carbon Black and FEP    | 0.45 |
| D2337                       | Water-borne Poly(amide-imide) w/ Carbon Black and FEP    | 0.35 |
| D2339                       | Water-borne Poly(amide-imide) w/ Carbon Black and FEP    | 0.5  |
| D2340 Xylan 1220/2810 Black | Water-borne Poly(amide-imide) w/ Carbon Black and FEP    | 0.25 |

## Example 4

Wire Testing Demonstrating Reduced V.O.C. Levels The use of the water-reducible polymer brings the level of solvents to a much lower volatile organic compound (V.O.C.) level, making the present coating formulation much more environmentally friendly than non water-reducible polymers. Testing of the above formulation was shown to provide V.O.C. levels of only about 4.4 lbs/gallon, as compared to a composition using non water-reducible poly (amide-imide)

## 14

formulation which demonstrated a significantly higher V.O.C. level of about 9.0 lbs/gallon. The formula for calculating VOC is shown below.

$$VOC = \frac{\text{Density (lb/gal)} \times (1 - \% \text{ Solids by Weight}) - \% \text{ Water by Weight}}{1 - \% \text{ Water by Volume}}$$

While the invention has been described in detail with reference to specific and preferred embodiments, it will be appreciated that various modifications and variations will be apparent to the artisan. All such modifications and embodiments as may readily occur to one skilled in the art are intended to be within the scope of the appended claims.

What is claimed is:

1. An improved apparatus for developing a latent image recorded on a surface, comprising:  
wire supports;  
a donor member spaced from the surface and being adapted to transport toner to a region opposed from the surface; and  
an electrode member positioned in the space between the surface and the donor member, the electrode member being closely spaced from the donor member and being electrically biased to detach toner from the donor member thereby enabling the formation of a toner cloud in the space between the electrode member and the surface with detached toner from the toner cloud developing the latent image, wherein opposed end regions of the electrode member are attached to said wire supports adapted to support the opposed end regions of said electrode member;  
wherein the improvement comprises applying to said non-attached regions of said electrode member, a coating composition comprising a water-emulsified polymer, a lubricant and an inorganic material.
2. An improved apparatus in accordance with claim 1, wherein said water-emulsified polymer is selected from the group consisting of water-emulsified acrylic, water-emulsified epoxy-phenolic, and water-emulsified poly(amide-imide).
3. An improved apparatus in accordance with claim 1, wherein said water-emulsified polymer is present in said coating composition in an amount of from about 25 to about 95 percent by weight of total coating composition.
4. An improved apparatus in accordance with claim 3, wherein said water-emulsified polymer is present in said coating composition in an amount of from about 50 to about 90 percent by weight of total coating composition.
5. An improved apparatus in accordance with claim 1, wherein said lubricant is selected from the group consisting of fluoroplastics, molybdenum disulfide, polyethersulfones, boron nitride, titanium diboride, graphite and mixtures thereof.
6. An improved apparatus in accordance with claim 5, wherein said fluoroplastic is selected from the group consisting of polytetrafluoroethylene, fluorinated ethylenepropylene copolymer, perfluorovinylalkylether tetrafluoroethylene copolymer, and mixtures thereof.
7. An improved apparatus in accordance with claim 6, wherein said fluoroplastic is fluorinated ethylene propylene.
8. An improved apparatus in accordance with claim 1, wherein said lubricant is present in said coating composition in an amount of from about 3 to about 50 percent by weight of total coating composition.
9. An improved apparatus in accordance with claim 8, wherein said lubricant is present in said coating composition

**15**

in an amount of from about 5 to about 25 percent by weight of total coating composition.

**10.** An improved apparatus in accordance with claim 1, wherein said inorganic material is an electrically conductive filler selected from the group consisting of metal oxides, 5 carbon black, graphite, surface treated carbon black, and mixtures thereof.

**11.** An improved apparatus in accordance with claim 10, wherein said electrically conductive filler is carbon black.

**12.** An improved apparatus in accordance with claim 1, 10 wherein said inorganic material is present in said coating composition in an amount of from about 5 to about 50 percent by weight of total coating composition.

**13.** An improved apparatus in accordance with claim 12, wherein said inorganic material is present in said coating 15 composition in an amount of from about 10 to about 25 percent by weight of total coating composition.

**14.** An improved apparatus in accordance with claim 1, wherein said composition is dip coated onto said electrode member.

**15.** An improved apparatus in accordance with claim 1, wherein said composition coating is present on from about 10 to about 90 percent of said electrode member.

**16.** An improved apparatus in accordance with claim 1, wherein said composition coating is of a thickness of from 25 about 1  $\mu\text{m}$  to about 5  $\mu\text{m}$ .

**17.** An improved apparatus in accordance with claim 1, wherein said electrode member includes at least one thin diameter wire.

**18.** An improved apparatus in accordance with claim 17, 30 wherein said at least one thin diameter wire has a diameter of from about 50 to about 100  $\mu\text{m}$ .

**19.** An improved apparatus in accordance with claim 1, wherein said electrode member is closely spaced from said donor member a distance of from about 0.001 to about 45 35  $\mu\text{m}$ .

**20.** An improved apparatus for developing a latent image recorded on a surface, comprising:

wire supports;

a donor member spaced from the surface and being 40 adapted to transport toner to a region opposed from the surface; and

an electrode member positioned in the space between the surface and the donor member, the electrode member being closely spaced from the donor member and being

**16**

electrically biased to detach toner from the donor member thereby enabling the formation of a toner cloud in the space between the electrode member and the surface with detached toner from the toner cloud developing the latent image, wherein opposed end regions of the electrode member are attached to said wire supports adapted to support the opposed end regions of said electrode member;

the improvement comprising applying to said non-attached regions of said electrode member, a coating composition comprising a) a water-emulsified polymer selected from the group consisting of water-emulsified acrylic, water-emulsified epoxy-phenolic, and water-emulsified poly (amide-imide); b) a fluorinated ethylene propylene lubricant; and c) carbon.

**21.** An improved electrostatographic process comprising:

a) forming an electrostatic latent image on a charge-retentive surface;

b) applying toner in the form of a toner cloud to said latent image to form a developed image on said charge-retentive surface, wherein said toner is applied using a development apparatus comprising wire supports; a donor member spaced from the surface and being adapted to transport toner to a region opposed from the surface; an electrode member positioned in the space between the surface and said donor member, said electrode member being closely spaced from said donor member and being electrically biased to detach toner from said donor member thereby enabling the formation of a toner cloud in the space between said electrode member and the surface with detached toner from the toner cloud developing the latent image, wherein opposed end regions of said electrode member are attached to said wire supports adapted to support the opposed end regions of said electrode member; wherein the improvement comprises applying to said non-attached regions of said electrode member, a water-emulsified polymer, a lubricant, and an inorganic material;

c) transferring the toner image from said charge-retentive surface to a substrate; and

d) fixing said toner image to said substrate.

\* \* \* \* \*